

## UNITED STATES PATENT OFFICE.

WARREN F. BLEECKER, OF BOULDER, COLORADO.

## METHOD OF PRODUCING AN IMPERVIOUS CHEMICAL MATERIAL.

No Drawing.

Application filed April 1, 1924. Serial No. 703,544.

My invention relates to impervious and chemically-resistant material and the method of its production and its principal object resides in providing a material suitable for 5 use in making pipe linings, conduits and machine parts, which is impervious to liquids and gases and proof against the corrosive action of acids and other chemicals and which owing to a high degree of tensile strength 10 and elasticity, is particularly adapted as a substitute for other materials heretofore used for similar purposes.

The material is of a composite character and its principal and essential constituent 15 elements are sulfur and a chemically-resistant body-forming substance, and it is a further object of the invention, to provide in the production of material of a molten mixture of the above stated substances, certain treatments which prevent the growth of large sulfur crystals and promote the formation of 20 small crystals desirably to or near the point of being amorphous, and which cause the particles and molecules of the ingredients to 25 be compacted so as to form a dense and substantially non-porous body devoid of voids and gas holes.

The treatments above referred to may consist in any action which decreases the cooling 30 period of the molten mixture, after it has been formed in the desired shape, to a point of solidification, or in any action productive of an intermolecular movement, and it should be understood that any two or more 35 of the above mentioned expedients may be combined for co-operative action, if so desired.

The methods for decreasing the cooling period 40 of the molten sulfur mixture and effecting an intermolecular movement in the same, may consist in rapidly cooling the mass by artificial means, in agitating or stirring the mass to a point of solidification, or in the proper application of pressure during the 45 cooling period, each action having for its purpose to separately or in conjunction with others, prevent the formation of large sulfur crystals and the occurrence of voids due to gasification of the molten sulfur, as hereinbefore explained.

An important function of the body giving

chemically-resistant substance intermixed with the sulfur, is to give to the material the necessary tensile strength, increase its elastic limits and decrease its co-efficient of expansion, and among the materials best suited for the purpose may be mentioned artificial graphite, sand, coke and pulverized slate, it being evident that the physical characteristics of the material may be varied by the use 55 of different substances of the above type, and that their selection is for this reason, governed to a large extent by the particular use or action for which the material or the article produced therefrom is intended and designed.

Inasmuch as artificial graphite is most suitable for the greater number of uses for which the material is intended, the following description will be limited to its employment with the understanding that other materials of the above described character may be substituted therefor in the same or different proportions according to varying requirements and within the scope of the 75 present invention.

An efficient method of reducing the solidification period of the molten sulfur mixture consists in rapidly cooling a surface with which the fluid mass engages, preferably 80 while the mass is under pressure, which causes the fluid matter to be compacted and restrained under gradual and progressive solidification.

In the production of pipe linings, the 85 above described action may be obtained by introducing the mixture in a molten condition into a pipe which is heated above the melting temperature and imparting to the pipe in a substantially horizontal position, a 90 revolving motion about its longitudinal axis, which forces the fluid material to the interior surface of the pipe under the influence of centrifugal force. While the pipe is thus revolved, its outer surface is cooled by any 95 suitable means such as a continuous application of cold water or other cooling fluid, with the result that the fluid matter is rapidly solidified progressively from its outer strata which engages with the surface of the pipe, 100 inwardly, while at the same time the inner portion of the liquid mass is continuously fed

to the cooling surface by the centrifugal pressure.

A microscopic examination of a lining thus produced, reveals a total absence of 5 large crystals and a compact arrangement of molecules without noticeable voids or crevices. In fact, the crystals are so small as to approach an amorphous condition and the formation is so dense as to be substantially 10 nonporous.

While the above method of forming conduits and pipe-linings of limited thickness is both practical and effectual, it will be evident that other means may be employed to 15 obtain a similar result and that in the production of machine parts of different character which do not permit of the employment of centrifugal force or of rapid cooling in the aforesaid manner, other methods must be 20 resorted to to obtain the required movement of the molecules in the fluid mixture and oppose the tendency of forming large crystals.

An effectual method of producing the desired result in the production of articles of 25 different forms and proportions consists in subjecting the liquid mass to an agitative or stirring action until it has cooled to a point of solidification. During this action artificial cooling means may be applied to 30 the matrix in which the material is formed, it being understood that in this method as well as in the first described process, rapid cooling of the material from one side to another is highly advantageous.

Different methods of subjecting the material to pressure while it cools in the required 35 form may be availed of where the employment of centrifugal force is not feasible or practical, and conduits or pipe-linings may 40 if so desired, be formed by ramming or pressing the fluid matter into a space between the pipe and a therewith concentric core and cooling the exterior surface thereof as before, or by pouring the molten mixture 45 into the pipe with a header of sufficient size to forcibly feed the liquid mass to the interior surface of the pipe during the cooling action.

The pressure to which the material is subjected, should always be sufficient to cause 50 the liquid portion of the material to enter into the pores of that which is already partially solidified by the cooling action upon the surface of the mold and that in the 55 formation of pipe-linings and conduits, it is advisable that their thickness should be maintained within certain definite limits on account of the poor conductivity of the sulfur mixture.

In all of the above described actions, the 60 exact nature of the mixture is of secondary consideration provided that it contains an adequate percentage of sulfur, it being evident that the character and proportions 65 of the other ingredients are subject to vari-

ation in accordance with different requirements.

What I claim and desire to secure by Letters Patent is:

1. The method of forming an impervious 70 chemically-resistant material consisting in subjecting a molten sulfur-mixture to an action causing intermolecular movement to a point of solidification.

2. The method of forming an impervious 75 chemically-resistant material consisting in artificially cooling a mixture of a chemically-resistant substance and molten sulfur.

3. The method of forming an impervious 80 chemically-resistant material consisting in artificially cooling a mixture of a chemically-resistant substance and molten sulfur, under pressure.

4. The method of forming an impervious 85 chemically-resistant material consisting in rapidly cooling a mixture of a chemically-resistant substance and molten sulfur, under pressure.

5. The method of forming an impervious 90 chemically-resistant material consisting in subjecting a molten sulfur-mixture upon a supporting surface to pressure, and artificially cooling said surface.

6. The method of forming an impervious 95 chemically-resistant material consisting in agitating a molten-sulfur mixture to a point of solidification.

7. The method of forming an impervious 100 chemically-resistant material consisting in agitating a molten-sulfur mixture to a point of solidification while the mixture is being artificially cooled.

8. The method of forming an impervious 105 chemically-resistant material consisting in artificially cooling a molten-sulfur mixture at one side thereof while being subject to pressure at its opposite side.

9. The method of forming an impervious 110 chemically-resistant material consisting in artificially cooling a molten-sulfur mixture at one side thereof while being subjected to centrifugal pressure at its opposite side.

10. The method of forming an impervious 115 and chemically-resistant hollow cylindrical body consisting in introducing into a revolving pipe, a molten sulfur-mixture and artificially cooling the exterior surface of the pipe.

11. The method of producing an impervious 120 chemically-resistant material consisting in subjecting a molten sulfur-mixture to an action accelerating the period of solidification during cooling.

12. The method of producing an impervious 125 chemically-resistant material consisting in subjecting a molten sulfur-mixture to an action opposing the formation of large sulfur crystals during cooling.

13. The method of producing an impervious 130 chemically-resistant material consist-

ing in subjecting a molten sulfur-mixture to pressure during cooling.

14. The method of producing an impervious chemically-resistant material consisting in artificially cooling a molten sulfur-

5 mixture while subjected to centrifugal pressure.

15. The method of producing an impervious chemically-resistant material consisting in artificially cooling a molten sulfur- 10 mixture while subjected to pressure.

In testimony whereof I have affixed my signature.

WARREN F. BLEECKER.